

Aug. 20, 1940.

H. L. KOHLER

2,212,269

PROTECTIVE COATED ARTICLE

Filed Nov. 9, 1938



Fig. 1



Fig. 2

INVENTOR  
HENRY L. KOHLER  
BY  
*Alfred R. Fuchs*  
ATTORNEY

## UNITED STATES PATENT OFFICE

2,212,269

## PROTECTIVE COATED ARTICLE

Henry L. Kohler, Kansas City, Mo., assignor to  
 Andrew A. Kramer, Kansas City, Mo.

Application November 9, 1938, Serial No. 239,670

6 Claims. (Cl. 29—181)

My invention relates to protective coated articles, and more particularly to sheet metal articles provided with a protective coating. This application is a continuation in part of my co-pending application Serial No. 144,029, filed May 21, 1937, patented March 21, 1939, Patent No. 2,150,929.

A difficulty that has always existed in the utilization of galvanized metallic sheets for making certain articles out of the same, has been that the galvanizing coating is not sufficiently resistant to corrosion under certain conditions to make the practical use thereof possible. An attempt to overcome this difficulty has been made by providing a heavier galvanizing coating on the sheet. The heavy zinc coating thus provided, however, has the disadvantage that, when the sheet is bent, the coating at the bend would crack and tend to peel or flake off. As a result, although the sheet as a whole was provided with a heavy galvanizing coating over its entire surface before being fabricated, the bending of a sheet to form a flange or a seam thereon, frequently damaged the galvanizing coating on the sheet so seriously that it would render the coating partially ineffective, on the outside of the bends required to form the flanges, or seams. Consequently the advantage of the heavy galvanizing coating on the sheet was largely lost, this being true because, at the point at which the galvanizing coating was caused to be damaged, or ruptured, by bending, the sheet would be, for practical purposes, no better than an uncoated sheet, as far as resistance to oxidization, or other corrosion, was concerned. While many attempts have been made to overcome this difficulty, by a hot dipping process after the article has been formed from the galvanized sheet, for example, this is difficult to accomplish and requires expensive equipment, if any large sheet metal article is to be galvanized after fabrication by such a dipping process.

It is a purpose of my invention to provide means for overcoming the above mentioned difficulty with galvanized sheets having a heavy coating of zinc thereon, and at the same time to provide a sheet that is more resistant to corrosion over the entire area thereof, if this is desired, than is possible with ordinary zinc coatings provided by a galvanizing process. I accomplish this by providing a mercury-zinc amalgam coating on the sheet, which is applied to any area thereof that may be desired.

My improved protective coating may be utilized to give better protection than zinc against cer-

tain types of corrosion, or corrosion due to certain causes, either over the entire area of a metallic sheet, or over the entire area of one side thereof, or over the entire area of a fabricated sheet metal section, or one side of such a section, if this should be desired, and is particularly adapted for use at and adjacent the bends in a fabricated sheet, whereby any rupture in the galvanizing coating that may have occurred during fabrication, from any of the fabrication steps, will be closed and the sheet protected at such bends, or other fabricated portions thereof, more effectively than was the case before the bending, or other operation, thereon, that damaged, or ruptured, the protective zinc coating on the sheet originally.

It is a further purpose of my invention to provide a protective coating of a zinc-mercury amalgam that has the same appearance as the zinc coating originally on the sheet as obtained by the galvanizing process. Galvanized metallic sheets have a characteristic spangled appearance. It is highly desirable to maintain this spangled appearance of the sheet after my improved coating has been placed thereon. This is accomplished by utilizing a paste-like zinc-mercury amalgam, which is applied to the sheet in a manner that the structural characteristics of the zinc coating on the sheet are not changed. My improved protective coating will resist every kind of corrosion equally as well, as does the galvanized sheet before having the treatment thereof, whereby my improved coating is produced, and for most uses, will produce a coating that will be more resistant to corrosion than the heavy galvanizing coating applied to such sheets, or fabricated sheet metal sections. As the term "fabrication" is used herein, it means any bending, cutting or punching operation, or any other operation on a sheet, that may be performed thereon after the same has been rolled and galvanized.

Other objects and advantages of my invention will appear as the description of the same proceeds. I desire to have it understood, however, that I do not intend to limit myself to the particular details described, except as defined in the claims.

In the drawing:

Fig. 1 is a fragmentary sectional view on a greatly enlarged scale, showing my improved amalgam coating applied to a sheet having a bend therein, and

Fig. 2 is a similar view, showing my improved

50

45

15

10

20

25

30

35

40

55

amalgam coating applied to a sheet otherwise fabricated than by bending.

Referring in detail to the drawing, in Figs. 1 and 2 the metallic body portion of the sheet, which is usually steel or iron, is indicated by the numeral 3. The sheet shown in Fig. 1 is bent at 4 and the bend may cause damage to the zinc coating ordinarily on the galvanized sheet on the outer side of the bend substantially at 10 the outer corner thereof. The zinc coating provided on the sheet is indicated by the numeral 5 and the amalgam coating around the outside of the bend and adjacent said bend in the sheet is indicated in Fig. 1 by the numeral 6.

15 In Fig. 2 the same numerals are applied to the zinc coating and the amalgam coating, but instead of showing a sheet with a bend therein, the sheet is shown as being fabricated by punching a hole 7 therein, this being merely illustrative 20 of some fabrication operation that may be performed on the sheet that may damage the ordinary zinc galvanizing coating thereon.

My improved protective coating is provided on galvanized sheets that have been fabricated to 25 the desired size and shape, by bending, die-shaping, cutting and punching operations, or any of these that may be necessary to produce the article, or sections of an article, of the desired shape from the galvanized sheet of metal. After the 30 sheet has been fabricated, it is cleaned at the places at which the protective coating is to be provided thereon, usually by means of dilute hydrochloric acid, or a solution of tin chloride, or antimony chloride, or lead chloride, or zinc chloride, or cyanide of soda. This cleaning solution 35 may be applied with a brush or swab of some character, and the excess may be removed with a cloth, or any other suitable means. When it is desired to apply the protective coating only at or adjacent 40 a ruptured area on a galvanized sheet, or an area that may have been damaged to the extent of injuring the protective coating, or rupturing the same, the galvanized sheets are cleaned only on the outer sides of all bends therein, or any 45 other area at which the coating may have been ruptured, or damaged, and areas adjacent these bends, or other areas where the damage may have occurred. A zone at the place at which the rupture 50 in the zinc coating may exist will thus be cleaned, and also a zone on each side thereof.

A putty-like amalgam of mercury and zinc is made up prior to cleaning the sheets, or is made up in quantity to be used whenever necessary, said amalgam having such proportions of zinc and 55 mercury therein as to produce a soft putty-like material of the consistency of thick paste or cream. The proportions of zinc and mercury that are used to produce this soft putty-like material will vary somewhat, dependent upon the atmospheric temperature existing, as the material must, 60 of course, be of the soft, creamy putty-like character at the temperature at which it is applied to the sheet. Thus in the winter time, when a lower temperature is encountered, both in the atmosphere and in the material of the sheets themselves, a larger proportion of the mercury to the zinc must be used to produce this soft putty-like coating material. I have found that 15% zinc and 85% mercury by weight will produce an 65 amalgam of the desired consistency in the summer time, while in the winter time, when the temperatures are exceedingly low, it is necessary to utilize an amalgam made for this purpose that will have as little as 10% zinc by weight, and 70 75 90% mercury by weight, while, if the mercury is

heated while the zinc is being incorporated therein, the percentage of zinc can be increased to 20% by weight to 80% by weight of mercury. The relative proportions of the metal, or metals, amalgamating with mercury that have to be utilized 5 depend upon the melting points of the metals that are amalgamated with mercury and the temperature encountered, and the heating makes it possible to incorporate a larger amount of the metal amalgamating with the mercury, than 10 would otherwise be the case. There is no advantage in incorporating too large a percentage of zinc in the amalgam, however, as it must, of course, remain of a creamy character, or a putty-like character, at the temperature at which it is 15 applied to the sheet, and if too large a percentage of zinc is included in the amalgam by adding the zinc to the heated mercury, it will not have the desired consistency at the temperature 20 at which it is to be utilized.

The zinc can be in the form of any small particles, such as shavings, turnings, cuttings, or in the form of a powder or granules. The finely divided zinc is stirred into the quantity of mercury that is to be utilized to make the amalgam 25 in the proportions necessary, substantially within the limits above referred to. This is ordinarily done without heating the mercury, but the mercury may be heated to incorporate a somewhat larger percentage of zinc in the amalgam than 30 would otherwise be possible within the limits pointed out above. Care must, of course, be utilized in doing this, that the mercury is not heated to a temperature near the vaporization 35 point thereof.

The soft putty-like amalgam of zinc and mercury, produced as above described, is applied to the cleaned zone, or area, of the galvanized sheet, by a brushing or rubbing operation, the soft putty-like amalgam being brushed or rubbed onto the cleaned area of the sheet with a cloth, or in a similar manner. This rubbing or brushing operation spreads the zinc-mercury amalgam over the cleaned area of the sheet and causes a thin layer 40 thereof to adhere to the outer surface of the zinc coating on the sheet. In case there is a rupture or a damaged area in the sheet, from which the zinc has been entirely, or substantially entirely, removed, the zinc-mercury amalgam will 45 adhere to the sheet at this ruptured area also. The amalgam, as soon as it contacts the zinc coating on the sheet, begins to act thereon to amalgamate the zinc on the sheet with some of the mercury in the amalgam. Due to the brushing of the amalgam back and forth over the ruptured area, the composition of the coating at the ruptured area will tend to be substantially the same as on other portions of the sheet to which the amalgam is applied. Any loose flakes, or particles, 50 of zinc will be dissolved in the amalgam, amalgamating with the mercury in said amalgam.

The action between the zinc-mercury amalgam and the zinc on the sheet will continue until the amalgam has penetrated the entire zinc coating of the sheet, at least down to the ferrous zinc alloy at the surface of the iron or steel of the sheet. After the zinc on the sheet amalgamates with the mercury, the resulting amalgam will 55 gradually become stiffer and harder, as the greater the amount of other metal amalgamated with the mercury the harder and stiffer the amalgam will become. As a result, the penetration of the zinc on the sheet by the zinc-mercury amalgam, will eventually produce a zinc-mercury amalgam throughout the coating on the sheet, 60 65 70 75 80 85 90 95

which will have lost the soft character that the zinc-mercury amalgam had when applied and will become as hard as the zinc coating originally on the sheet.

5 Thus, while the amalgam, when first placed on the sheet, will be soft enough that it can be rubbed off on the fingers to a certain extent, after at least twenty-four hours, the coating at the area to which the amalgam has been applied 10 will be hard enough that none of the same will rub off and the sheet can be handled without any damage to the coating thereon, just as readily as was the case with the zinc coating on the sheet originally. The sheet will, after the coating 15 has become hard, have substantially the same appearance as it did before any amalgam was applied thereto, and none of the coating can be rubbed off, even though it may be rubbed persistently for a considerable period of time. The 20 coating will have the characteristic spangled appearance of the zinc coating originally on the sheet. This indicates that the application of the putty-like amalgam to the sheet that has been previously galvanized, while resulting in the 25 dissolving of the zinc on the sheet, in the mercury of the amalgam, does this in such a gradual manner that the liquefaction of the coating material on the sheet takes place at such a slow rate through the thickness of the zinc coating, that 30 the structure of the zinc coating on the sheet is not altered, although the composition changes from substantially pure zinc to a zinc-mercury amalgam, as the amalgamating process proceeds through the coating. The sheet will accordingly 35 have substantially the same appearance two or three days after the amalgam was applied thereto as it had before any application of amalgam thereto.

It is obvious that it may be desirable to not 40 only prevent corrosion at ruptures in coatings on galvanized sheets at bends in such sheets, or similar places, but that the entire area of a sheet, or the entire inner surface of a sheet, or section of a container, for example, that is innermost 45 when it is in place, and which is subjected to the corrosive action of sulphuric acid, or other compounds, which are ordinarily found in oil tanks, or similar receptacles, may be provided with a corrosion resisting amalgam coating. By utilizing 50 my protective coating, the corrosive action, caused by these sulphur compounds, on the zinc coating of the sheet ordinarily occurring will be reduced and substantially eliminated, the zinc-mercury amalgam being applied to the inner 55 surface of such oil tank, or the sections of such an oil tank, made up of sheets that have been bent, cut and punched before the application of the amalgam thereto.

The tendency of the sulphur compounds, when 60 acting on the amalgam coating described, is to cause the mercury in the amalgam to form a protective film on the surface that is exposed to the action of the dilute sulphuric acid, or hydrogen sulphide, or other sulphur compounds, this causing 65 some slight loss of some of the zinc, but the mercury arresting this substantially immediately, due to its film forming action.

While it is immaterial whether the amalgam 70 coating is of the same composition throughout, it has been found that if the soft putty-like amalgam, above referred to, is utilized, some of the mercury in the amalgam will amalgamate with the zinc immediately, forming a zinc-mercury amalgam, and some of the zinc-mercury amalgam will be present in substantially the form in

which it was applied at first, this being on the top surface of the coating. However, if the amalgam above referred to is left in contact with the zinc coating for twenty-four hours or more, and an excessive amount of the amalgam is not 5 used, sufficient of the mercury will amalgamate with the zinc that all of the zinc will become amalgamated with the mercury, and the resulting coating will be a zinc-mercury amalgam from the outer surface of the coating to at least the ferrous 10 zinc alloy at the surface of the metal of the sheet. The amalgamation of the mercury with the zinc on the sheet, when completed, causes the coating to have a hard character, because there is so much larger a percentage of zinc in 15 the coating, than there was in the amalgam applied to the sheet, and the coating will have a hard character, similar to that of the zinc, instead of a soft putty-like character, such as the zinc-mercury amalgam, that was applied to the 20 sheet, had at the time of application.

When a putty-like amalgam, containing 15% zinc and 85% mercury by weight, is utilized for application to a galvanized sheet that has a zinc coating thereon amounting to one ounce per running square foot, or one-half ounce per square foot running surface on each side of the sheet, the amalgam resulting will contain approximately 90% zinc and 10% mercury. With heavier coatings of zinc, the percentage of zinc will, of course, 25 be higher. Thus zinc coatings as thick as two and one-half ounces per running square foot, have been utilized on galvanized sheets, and for such coatings the resulting amalgam on the sheet will contain about 95.6% zinc, and 4.4% 30 mercury. The putty-like amalgam is applied only thick enough to completely coat the sheet and, of course, with a heavier zinc coating the resulting amalgam would contain a much smaller 35 percentage of mercury than where sheets with lighter coatings of zinc are treated to produce my improved amalgam coating. As some variation can also be practiced in the percentages of zinc or mercury in the putty-like amalgam, depending upon temperature conditions, it has 40 been found that the amount of zinc can be varied between 10% and 20% and said putty-like coating materials produced for application to the sheet to produce the amalgam that eventually 45 is formed on said sheet. Due to these variations, the percentage of zinc finally on the sheet where the amalgam coating is provided thereon will 50 range between 89% and 96%, while the percentage of mercury will range between 11% and 4%. In all cases, the amalgam resulting that is 55 on the sheet will contain well over 50% zinc and the coating will not lose the characteristics of a zinc coating, except in part, but will be modified to some extent in its characteristics by the mercury contained therein, the mercury acting to 60 make the coating more resistant to corrosion than the zinc coating was originally. Such a zinc mercury amalgam coating on a sheet is particularly desirable where it is preferred that no lead, or tin, or other metal than zinc and mercury, 65 be present on the surface of the sheet. While the zinc will tend to dissolve under the same circumstances in which it would dissolve on an ordinary galvanized sheet, in a sheet that is provided with an amalgam coating, such as described herein, the mercury in the amalgam acts to arrest this action on the zinc and causes the zinc-mercury amalgam coating to have a much longer life than a pure zinc coating would have.

It is highly desirable that the spangled appear- 75

5 ance of the coating on the sheet, such as it has when galvanized, be maintained, as this coating has a desirable appearance from the standpoint of the user, and due to the familiarity of the user with the spangled appearance of galvanized sheets, any destruction of this appearance is found to be objectionable from a commercial standpoint.

What I claim is:

- 10 1. A galvanized sheet having a coating of zinc and mercury containing from eight to sixteen parts of zinc to one part of mercury by weight on one side thereof, said coating having at least as great a proportion of mercury at its exposed surface as adjacent the metal of the sheet.

15 2. A galvanized sheet having a bend therein and having a coating of zinc and mercury containing from eight to sixteen parts of zinc to one part of mercury by weight on the side thereof lying on the outside of said bend at and adjacent said bend, said coating having at least as great a proportion of mercury at its exposed surface as adjacent the metal of the sheet.

20 3. A galvanized sheet having a mercury-zinc amalgam coating on one side thereof, having at least as great a proportion of mercury at its exposed surface as adjacent the metal of the sheet, said coating having a much greater proportion of zinc than mercury therein.

4. A galvanized sheet having a bend therein and having a mercury-zinc amalgam coating on the inside thereof lying on the outside of said bend at and adjacent said bend, said coating having at least as great a proportion of mercury at its exposed surface as adjacent the metal of the sheet and having a much greater proportion of zinc than mercury therein.

5. A fabricated steel sheet having a zinc galvanizing coating therein, said zinc coating having interruptions therein, and a zinc-mercury amalgam coating thereon over and adjacent the interruptions in said zinc coating, said amalgam coating having at least as great a proportion of mercury at its exposed surface as adjacent the metal of the sheet and having a much greater proportion of zinc than mercury therein.

6. A galvanized metallic sheet having a zinc coating on a portion of the area thereof and a coating of an amalgam composed of zinc and mercury on the remainder of the area thereof, said amalgam coating having at least as great a proportion of mercury at its exposed surface as adjacent the metal of the sheet and having a much greater proportion of zinc than mercury therein.

HENRY L. KOHLER.